

# UNITED STATES PATENT OFFICE.

GEORGE A. HENDERSON, OF ST. ALBANS, WEST VIRGINIA.

## FIBROUS COMPOSITION AND PROCESS FOR MAKING THE SAME.

1,270,732.

Specification of Letters Patent. Patented June 25, 1918.

No Drawing. Original application filed November 30, 1915, Serial No. 64,285. Divided and this application filed July 30, 1917. Serial No. 183,598.

*To all whom it may concern:*

Be it known that I, GEORGE A. HENDERSON, a citizen of the United States, residing at St. Albans, in the county of Kanawha, 5 State of West Virginia, have invented a new and useful Improvement in Fibrous Composition and Processes for Making the Same, of which the following is a full, clear, and exact description.

10 The primary object of the invention is the effective and uniform impregnation of woody particles, formed of a plurality of wood fibers, with a preservative material of a binding nature for producing a durable 15 and efficient compound especially well adapted for paving and like purposes.

A further object of the invention is to insure permanent density of the product of the process by the removal of the cellular 20 tissue, sap, and softer portion of the wood by destructive distillation thereof, and by strong heat applied thereto during the impregnation of the remaining fibers with a preservative binder.

25 In carrying out my invention, I provide for the shredding of this waste material from hardwood into particles of uniform thickness, but of irregular length and breadths, and of various sizes ranging from 30 particles just larger than impalpable dust up to three quarters of an inch in length, and of lesser breadth, and then grading the sizes of the woody particles so that the smaller particles will as nearly as may be, fill the

35 voids between the larger ones; then agitating and conveying the same through hot bitumen in predetermined quantity only sufficient to coat, and to fill the pores of the particles, and the voids between the par-

40 ticles, and to bind them together in an open ended vat under sustained heat to expand the particles and to expel the moisture and sap, and to destroy the cellular tissue and other softer portion of the wood, thus ren-

45 dering the particles susceptible to their maximum capacity to impregnation by absorption of the bitumen, simultaneously drawing the vapors out of the vat, removing the material from the vat, and then while 50 cooling and contracting, compressing the mass into shape.

In a modification of my invention the material may be allowed to cool, after being removed from the aforesaid vat, in which 55 event the same shall be re-heated, and while

hot, removed from the re-heater, and while cooling and contracting it shall be compressed into shape.

In a further modification of my invention, the sap and tissues may be first removed 60 from the particles by cooking the same, or by other methods known to extract manufacturers, and the trade; and some of the excess moisture may be removed from the comminuted, of shredded particles, by heat 65 or otherwise, before mixing the bitumen therewith.

I claim:

1. The process of treating fibrous vegetable material, forming comminuted fibrous 70 particles of exactly uniform thickness but of irregular lengths and breadths, expanding the particles by conveying the same through an open ended vat containing hot binding and preservative agent to expand 75 the pores of the fiber, and to convert the remaining moisture in the particles into steam and to impregnate the pores of the material with a binding preservative agent, 80 the quantity of which shall be predetermined by measuring and mixing a portion of the ingredients together in such manner that there is present merely sufficient preservative-binder to fill the pores of the vegetable material, to coat the particles thereof, 85 to fill the voids between the particles and to bind them to each other, drawing the steam vapors out of the vat during said impregnation, and then compressing the material into shape. 90

2. In a process of treating fibrous vegetable material forming comminuted fibrous particles of hard wood of exactly uniform thickness, but of irregular lengths and breadths, grading the sizes of said particles 95 from just larger than impalpable dust up to three quarters of an inch in length, and mixing percentages of each size of said particles so that the smaller ones will, as nearly as may be, fill the voids between the larger 100 particles; then conveying the same through an open ended vat to heat the same, then depositing the same into a hot binding preservative agent within the vat, and agitating the same a sufficient length of time to 105 expel from the particles all remaining moisture, and to abnormally enlarge and expand the pores of the particles, to impregnate the same with a predetermined quantity of binding preservative agent, only sufficient in 110

quantiy to completely fill the pores within the fibrous particles, in their subsequently contracted compressed condition, to surround the particles, and fill the voids between the same, in the final product, and to bind the particles together; then while hot, removing the material from the vat, and while cooling compressing the same into shape.

- 10 3. In a process of treating fibrous vegetable material, forming comminuted fibrous particles of uniform thickness, but of irregular lengths and breadths, subjecting the same to a cooking operation, then extracting the moisture from the material while hot, then conveying the material through an open ended vat containing hot binding and preservative agent, to convert the remaining moisture in the material into steam and to impregnate the pores of the material with the binding and preservative agent, drawing steam vapors out of the vat during said impregnation, and pressing the same into shape.
- 15 4. In a process of treating fibrous vegetable material, forming comminuted fibrous particles of uniform thickness but of irregular lengths and breadths, clearing the pores or interstices of the particles of sap and like soft materials, expanding the pores by heat, impregnating the expanded pores with a preservative agent while the pores are expanding, then contracting the particles by cooling the mass; then compressing the same while contracting into shape.
- 20 5. A plastic composition of hard-wood particles of uniform thickness, and of irregular lengths and breadths, from which sap, cellular tissue and moisture have been removed, impregnated with a preservative-binder and pressed into shape.

table material, forming comminuted fibrous particles of exactly uniform thickness but of irregular length and breadths, clearing the pores or interstices of the particles of sap and like soft materials, expanding the pores by heat, impregnating the expanded pores with a preservative agent while the pores are expanding, then contracting the particles by cooling the mass; then compressing the same while contracting into shape.

5. A plastic composition of hard-wood particles of uniform thickness, and of irregular lengths and breadths, from which sap, cellular tissue and moisture have been removed, impregnated with a preservative-binder and pressed into shape.

In testimony whereof I have affixed my signature in the presence of two witnesses, the twenty-seventh day of July, 1917.

GEORGE A. HENDERSON.

Witnesses:

R. H. MAGUIRE,  
LENICE HATFIELD.